# EUROPEAN PATENT SPECIFICATION

(11) **EP 3 852 199 B1**
(45) Date of publication and mention of the grant of the patent: **30.08.2023**
(21) Application number: 19861121.2
(22) Date of filing: 10.09.2019
(51) Int. Cl.: H01R 13/405, H01R 13/53, H01R 13/74, H01R 13/03, H01R 13/504

(54) **HERMETIC TERMINAL**
HERMETISCHES ANSCHLUSSELEMENT
BORNE HERMÉTIQUE

(30) Priority: 11.09.2018 JP 2018169868
(43) Date of publication of application: 21.07.2021
(73) Proprietor: Kyocera Corporation, Kyoto-shi, Kyoto 612-8501 (JP)
(72) Inventor: OOMURA,Haruka, Kyoto-shi, Kyoto 612-8501 (JP); IWAMOTO,Koichi, Kyoto-shi, Kyoto 612-8501 (JP)
(74) Representative: Viering, Jentschura & Partner mbB Patent- und Rechtsanwälte
(86) International application number: PCT/JP2019/035503
(87) International publication number: WO 2020/054703

(56) References cited:
- WO-A1-2011/096592
- JP-A- H07 282 621
- JP-A- 2005 235 576
- JP-A- 2005 235 577
- JP-A- 2006 179 340
- JP-A- 2006 324 229
- JP-A- 2007 201 335
- JP-B2- 2 519 642
- JP-U- H04 119 964
- JP-Y2- H0 212 682

## Description

### TECHNICAL FIELD

The present disclosure relates to a hermetic terminal.

### BACKGROUND

Conventionally, in hermetic terminals used in a vacuum equipment, a nuclear equipment, or the like, a contact pin 21, a heat-resistant insulator 22, and a pipe flange (tube body) 23 are hermetically connected to each other as a hermetic terminal 30 shown in Fig. 5 to obtain a high leakage resistance, and the connecting is performed by brazing or the like, and it is required to have a necessary mechanical strength, and withstand impact and high temperature sufficiently. Therefore, alumina is used as the heat-resistant insulator 22, its surface is metallized, it is hermetically connected to the contact pin 21 and the pipe flange 23 by brazing, and to reduce difference of thermal expansion coefficients of the contact pin 21 and the pipe flange 23 with respect to the alumina, the contact pin 22 and the pipe flange 23 are normally formed by an iron-nickel alloy or an iron-nickel cobalt alloy.

Further, recently, as shown in Non-Patent Document 1, a multi-pole terminal is used as a hermetic terminal for extracting signal of a liquid hydrogen tank of a rocket.

### PRIOR ART DOCUMENTS

### Patent Document

Patent Document 1: Japanese Patent Publication No. 2519642

Another patent document, JP2005235577A, discloses a hermetic terminal according to the preamble of claim 1.

### Non-Patent Document

Non-Patent Document 1: Hajime Ishimaru, Hermetic Seal for Low Temperature, TEION KOGAKU 17(1), pp. 61-62 (1982)

### SUMMARY

A hermetic terminal of the present disclosure includes a plate-shaped ceramic substrate in a plate shape provided with a through hole for inserting a columnar conductive member in a thickness direction, a first tube body surrounding the ceramic substrate, and a second tube body coaxially connected with the first tube body , and the first tube body includes a fernico-type alloy, an Fe-Ni alloy, an Fe-Ni-Cr-Ti-Al alloy, an Fe-Cr-Al alloy or an Fe-Co-Cr alloy, and the second tube body includes an austenitic stainless steel with a nickel content of 10.4 mass% or more.

### BRIEF DESCRIPTION OF THE DRAWINGS

FIG. 1(a) is a perspective view at a side of a first tube body, and FIG. 1(b) is a perspective view at a side of a second tube body, illustrating one embodiment of a hermetic terminal of the present disclosure.
FIG. 2(a) is a drawing illustrating one embodiment of a sectional view along an axis direction of the first tube body and the second tube body, FIG. 2(b) is a side view of FIG. 2(a), FIG. 2(c) is a sectional view illustrating one embodiment enlarging the part A shown in FIG. 2(a), FIG. 2(d) is a sectional view illustrating another embodiment enlarging the part A shown in FIG. 2(a), and FIG. 2(e) is a sectional view illustrating one embodiment enlarging the part B shown in FIG. 2(a), illustrating the hermetic terminal of FIG. 1.
FIG. 3 is a sectional view illustrating another embodiment enlarging the part A of the hermetic terminal shown in FIG. 2.
FIG. 4(a) is a drawing illustrating another embodiment of a sectional view along the axis direction of the first tube body and the second tube body, FIG. 4(b) is a side view of FIG. 4(a), FIG. 4(c) is a sectional view illustrating one embodiment enlarging the part A shown in FIG. 4(a), FIG. 4(d) is a sectional view illustrating another embodiment enlarging the part A shown in FIG. 4(a), and FIG. 4(e) is a sectional view illustrating one embodiment enlarging the part B shown in FIG. 4(a), illustrating the hermetic terminal of FIG. 1.
FIG. 5 is a perspective view illustrating one embodiment of a conventional hermetic terminal.

### EMBODIMENT

Embodiments of the present invention are described in detail below with reference to the drawings. In all the drawings of the present description, the same parts are designated by the same reference numerals unless confusion occurs, and the description thereof will be omitted as appropriate.

FIG. 1(a) is a perspective view at a side of a first tube body, and FIG. 1(b) is a perspective view at a side of a second tube body, illustrating one embodiment of a hermetic terminal of the present disclosure.

FIG. 2(a) is a drawing illustrating one embodiment of a sectional view along an axis direction of the first tube body and the second tube body, FIG. 2(b) is a side view of FIG. 2(a), FIG. 2(c) is a sectional view illustrating one embodiment enlarging the part A shown in FIG. 2(a), FIG. 2(d) is a sectional view illustrating another embodiment enlarging the part A shown in FIG. 2(a), and FIG. 2(e) is a sectional view illustrating one embodiment enlarging the part B shown in FIG. 2(a), illustrating the hermetic terminal of FIG. 1.

A hermetic terminal 20 illustrated in FIGs. 1 and 2 includes a plate shape ceramic substrate 3 provided with a through hole 2 for inserting a columnar conductive member 1 in a thickness direction, a first tube body 4 surrounding the ceramic substrate 3, and a second tube body 5 coaxially connected with the first tube body 4.

The conductive member 1 includes a columnar base part 1a inserted into the through hole 2, and a collar part 1b opposing to the ceramic substrate 3 on the midway in an axis direction of the columnar base part 1a. The conductive member 1 includes a fernico-type alloy, an Fe-Ni alloy, an Fe-Ni-Cr-Ti-Al alloy, an Fe-Co-Cr alloy or an Fe-Cr-Al alloy, the ceramic substrate 3 includes ceramics including aluminum oxide as a main component, and the conductive member 1 is supported by the ceramic substrate 3 provided with a metallized layer 10 formed on the surface by a brazing material including silver such as BAg-8, BAg-8A, BAg-8B or the like as a main component.

The term "main component in the ceramics" denotes a component of 85 mass% or more in 100 mass% of the components constituting the ceramics, the term "main component in the brazing material" denotes a component of 60 mass% or more in 100 mass% of the components constituting the brazing material.

The ceramics may include at least one of silicon, calcium and magnesium as an oxide in addition to aluminum oxide which is a main component.

The components constituting the ceramics may be identified by using an X-ray diffractometer (XRD), and then the content of components may be determined by using an X-ray fluorescent analyzer (XRF) or an ICP emission spectrometer (ICP), and converted it into the content of the identified components.

The content of the components constituting the brazing material may be determined by using an X-ray fluorescent analyzer (XRF) or an ICP emission spectrometer (ICP).

The first tube body 4 includes a shaft part 4a and a head part 4b having an outer diameter larger than the outer diameter of the shaft part 4a. Similarly, the second tube body 5 includes a shaft part 5a and a head part 5b having an outer diameter larger than the outer diameter of the shaft part 5a.

The hermetic terminal 20 includes a flange 6 provided with a plurality of through holes 6a for inserting the second tube body 5, and a plurality of through holes 6b for inserting fastening members such as bolts or the like on the outer peripheral side to fix a storage container for low temperature liquid or the like (not shown). The flange 6, for example, includes an austenitic stainless steel.

As shown in FIG. 2(a), the flange 6 surrounds the shaft part 4a of the first tube body 4 and the shaft part 5a of the second tube body 5, and separates an environment different on the left and right sides with the flange 6 as a boundary.

In FIG. 2(a), the side of the head part 4b of the head part 4b and the shaft part 4a of the first tube body 4 located on the left side of the ceramic substrate 3 is used in an environment exposed to the atmosphere, the second tube body 5 located on the right side of the ceramic substrate 3 is used in an environment exposed to liquid hydrogen. The shaft part 4a of the first tube body 4 located on the right side of the ceramic substrate 3 is configured not to be directly exposed to the liquid hydrogen by the second tube body 5.

The first tube body 4 includes a fernico alloy, an Fe-Ni alloy, an Fe-Ni-Cr-Ti-Al alloy, an Fe-Cr-Al alloy or an Fe-Co-Cr alloy, and the second tube body 5 includes an austenitic stainless steel with a nickel content of 10.4 mass% or more.

If the first tube body 4 includes the above-described alloys, even if heating and cooling are repeated, linear expansion coefficients of these alloys have a small difference from a linear expansion coefficient of aluminum oxide, so residual stress is less likely to accumulate in the ceramic substrate 3, and thus cracks are less likely to occur in the ceramic substrate 3. Additionally, if the second tube body 5 includes the austenitic stainless steel with the nickel content of 10.4 mass% or more, it is less likely to be embrittled by hydrogen and can therefore be used for a long period of time.

The second tube body 5 includes, for example, SUS310S, SUS316L, SUS316LN, SUS316J1L or SUS317L.

In FIGs. 1 and 2, the first tube body 4 and the second tube body 5 are both circular cylindrical bodies, and the ceramic substrate 3 is a disk, but the first tube body 4 and the second tube body 5 may be both square cylindrical bodies, and the ceramic substrate 3 may be a square plate.

As shown in FIG. 2(c), an end of the second tube body 5 on the side of the first tube body 4 includes a step surface 5c.

As shown in FIG. 2(d), an end of the first tube body 4 on the side of the second tube body 5 includes a step surface 4c.

As shown in FIGs. 2(c) and 2(d), at least one of the end of the second tube body 5 on the side of the first tube body 4 and the end of the first tube body 4 on the side of the second tube body 5 may include the step surfaces 4c and 5c. In FIG. 2(c), the step surface 5c is included on the outer peripheral surface of the second tube body 5, but the step surface may be included on the inner peripheral surface of the second tube body 5. Additionally, in FIG. 2(d), the step surface 4c is included on the outer peripheral surface of the first tube body 4, but the step surface may be included on the inner peripheral surface of the first tube body 4.

With such a configuration, hydrogen volatilized by applying a high pressure is difficult to pass through a gap between the first tube body 4 and the second tube body 5, so that the volatilized hydrogen becomes difficult to leak to the outside through an internal space of the first tube body 4.

FIG. 3 is a sectional view illustrating another embodiment enlarging the part A of the hermetic terminal shown in FIG. 2.

As shown in FIG. 3, the second tube body 5 may include a coating layer 5d composed of nickel, copper or a copper-nickel alloy as a main component at least on a connecting part with the first tube body 4.

With such a configuration, the first tube body 4 and the second tube body 5 can be connected firmly by a connecting layer 7 including a brazing material, and thus reliability is improved.

The second tube body 5 may include the coating layer 5d composed of nickel, copper or a copper-nickel alloy as a main component on at least one of the surfaces exposed to the liquid hydrogen such as the inner peripheral surface, the outer peripheral surface, and the end surface in addition to the connecting part.

With such a configuration, embrittlement due to hydrogen of the austenitic stainless steel constituting the second tube body 5 can be delayed, so that it can be used for a longer period of time.

The second tube body 5 shown in FIG. 3 includes the coating layer 5d on the inner peripheral surface, the outer peripheral surface, and the end surface.

The first tube body 4 may include a coating layer 4d composed of nickel, copper or a copper-nickel alloy as a main component at least on a connecting part with the second tube body 5.

With such a configuration, the first tube body 4 and the second tube body 5 can be connected firmly by a brazing material, and thus reliability is improved.

As shown in FIG. 3, the inner peripheral surface of the first tube body 4 may be located outward rather than the outer peripheral surface of the second tube body 5.

With such a configuration, the first tube body 4 has a linear expansion coefficient smaller than the second tube body 5, so the gap is less likely to expand even if heating and cooling are repeated, and thus the volatilized hydrogen is less likely to leak to the outside through the internal space of the first tube body 4.

As shown in FIG. 3(a), if the second tube body 5 includes the step surface 5c on the end of the second tube body 5 on the side of the first tube body 4, the outer peripheral surface corresponds to the step surface 5c.

As shown in FIGs. 1 and 2, the flange 6 connected to the outer peripheral surface of the second tube body 5 and surrounding the second tube body 5 may be further included.

With such a configuration, different environments can be separated on the outer peripheral side of the second tube body 5 with the flange 6 as a boundary.

Then, as shown in FIG. 2, the flange 6 includes a second recessed part 6d at the side of the second tube body 5, a collar part 8 having a U-shaped cross section along an axial direction of the second tube body 5 is attached to the second recessed part 6d, and the second tube body 5 and the flange 6 are connected via the collar part 8.

The collar part 8 may include a coating layer (not shown) including nickel, copper or a copper-nickel alloy as a main component at least on the connecting part with the second tube body 5, and the coating layer (not shown) may be included on entire surface of the collar part 8.

The term "main component in the coating layer" in the present disclosure denotes a component of 88 mass% or more in 100 mass% of the components constituting the coating layer, and may include phosphorus or the like in addition to the main component. If the coating layer including the copper-nickel alloy as a main component, the total content of copper and nickel is the content of the main component.

The content of the components in the coating layer may be determined by using an X-ray fluorescent analyzer (XRF) or an ICP emission spectrometer (ICP).

The collar part 8 and the second tube body 5 are connected by the brazing material including silver such as BAg-8, BAg-8A, BAg-8B or the like as a main component, and the flange 6 and the collar part 8 are welded by a TIG (Tungsten Inert Gas) welding method, and this welding is performed after each member is connected with the brazing material.

The flange 6 includes a first recessed part 6c at the side of the first tube body 4, and it is preferable that the connecting part between the ceramic substrate 3 and the first tube body 4 is located away from the second tube body 5 than a bottom surface 6c1 of the first recessed part 6c (that is, in FIG. 2(a), it is preferable that the connecting part between the ceramic substrate 3 and the first tube body 4 is located on the left side of the drawing with respect to a virtual plane where the bottom surface 6c1 of the first recessed part 6c is located, and the second tube body 5 is located on the right side of the drawing with respect to the virtual plane).

If the connecting part between the ceramic substrate 3 and the first tube body 4 is at this position, the heat generated by welding is less likely to be transferred to the ceramic substrate 3, so that residual stress is less likely to be generated in the ceramic substrate 3, and cracks are less likely to occur in the ceramic substrate 3.

Here, the first recessed part 6c is a counterbore for facilitating the attachment of the first tube body 4.

Further, the collar part 8 may include the austenitic stainless steel with the nickel content of 10.4 mass% or more. If the collar part 8 has such a configuration, it is less likely to be embrittled by hydrogen and can therefore be used for a long period of time.

The collar part 8 includes, for example, SUS310S, SUS316L, SUS316LN, SUS316J1L or SUS317L.

The nickel content in the second tube body 5 and the collar part 8 can be measured by using an ICP (Inductively Coupled Plasma) emission spectrometer or an X-ray fluorescent analyzer (XRF).

FIG. 4(a) is a drawing illustrating another embodiment of a sectional view along the axis direction of the first tube body and the second tube body, FIG. 4(b) is a side view of FIG. 4(a), FIG. 4(c) is a sectional view illustrating one embodiment enlarging the part A shown in FIG. 4(a), FIG. 4(d) is a sectional view illustrating another embodiment enlarging the part A shown in FIG. 4(a), and FIG. 4(e) is a sectional view illustrating one embodiment enlarging the part B shown in FIG. 4(a), illustrating the hermetic terminal of FIG. 1.

As shown in FIG. 4, a plurality of conductive members 1 are individually inserted into a plurality of through holes 2, and the ceramic substrate 3 includes step parts 9 (9a, 9b) recessed from at least one of the main surfaces 3b, 3c around the through holes 2.

With such a configuration, a creepage distance between columnar base parts 1a of the conductive members 1 adjacent to each other becomes long, so that generation of creepage discharge between the columnar base parts 1a can be suppressed.

The ceramic substrate 3 includes the step parts 9 recessed from both of the main surfaces 3b, 3c around the through holes 2, and one of the step parts 9a further includes a metallized layer 10 on the step surface, and the step part 9a on the side provided with the metallized layer 10 may be deeper than the step part 9b on the side not provided with the metallized layer 10. Here, the metallized layer 10 is for fixing the conductive member 1 to the ceramic substrate 3 by brazing, and the thickness thereof is, for example, 5 um or more and 55 um or less.

If the step part 9a on the side provided with the metallized layer 10 is deeper than the step part 9b on the side provided with the metallized layer 10, the creepage distance between the columnar base parts 1a of the conductive members 1 adjacent to each other can be lengthened, so that even if the metallized layer 10 is made thicker, generation of creepage discharge between the conductive members 1 can be suppressed. Here, the depth of the step part 9a is a distance from the main surface to the step surface, and it does not include the thickness of the metallized layer 10.

The depth of the step part 9a on the side provided with the metallized layer 10 may be 45% or less of the thickness of the ceramic substrate 3. If the depth of the step part 9a is in this range, mechanical strength of the ceramic substrate 3 around the through holes 2 can be ensured. Here, the thickness of the ceramic substrate 3 is a distance between both main surfaces 3b, 3c of the ceramic substrate 3.

Further, as shown in FIG. 2, the plurality of conductive members 1 are individually inserted into the plurality of through holes 2, and the ceramic substrate 3 includes a protrusion part 3a extending from at least one of the main surfaces (the main surface 3c in the example shown in FIG. 2) around the through holes 2. With such a configuration, the metallized layer 10 opposing to the conductive member 1 can be lengthened, so that reliability of the connecting of the conductive member 1 to the ceramic substrate 3 can be increased.

The ceramic substrate 3 includes a plurality of open pores on the step surface where the metallized layer 10 is included or the tip end surface of the protrusion part 3a, and the value obtained by subtracting an average value of the equivalent circle diameters of the open pores from the distance between the centers of gravity of the open pores may be 20 um or more and 50 um or less.

If the value obtained by subtracting the average value of the equivalent circle diameters of the open pores from the distance between the centers of gravity of the open pores is 20 um or more, it becomes difficult for the open pores to communicate with each other even if used in an environment where heating and cooling are repeated, so that the mechanical strength can be maintained, and cracks are less likely to occur in the metallized layer 10. Further, if the value obtained by subtracting the average value of the equivalent circle diameters of the open pores from the distance between the centers of gravity of the open pores is 50 um or less, the density of the open pores is increased, so that an anchor effect of the metallized layer 10 to the ceramic substrate 3 is improved, and adhesion strength of the metallized layer 10 is increased.

If the value obtained by subtracting the average value of the equivalent circle diameters of the open pores from the distance between the centers of gravity of the open pores is 20 um or more and 50 µm or less, the mechanical strength of the ceramic substrate 3 can be maintained, cracks can be suppressed in the metallized layer 10, and the adhesion strength of the metallized layer 10 can be improved.

In case of obtaining the distance between the centers of gravity of the open pores, the step surface of the ceramic substrate 3 or the tip end surface of the protrusion part 3a is polished with diamond abrasive grains to obtain a mirror surface. Here, an arithmetic mean roughness Ra of the mirror surface is set to 0.2 um or less by using a measurement method in accordance with JIS B 0601: 2013. A part where the size and distribution of the open pores are observed on average is selected from the mirror surface, and an optical microscope is used with a magnification of 200 times to measure an area of, for example, 1.5 × 10⁵ µm² as a measurement area.

By using the measurement area as a measurement object, a method called a distance between centers of gravity of an image analysis software "A-ZOKUN (ver 2.52)" (registered trademark, produced by Asahi Kasei Engineering Corporation, and hereinafter, indicated by the image analysis software) is applied, and the distance between the centers of gravity of the open pores adjacent to each other can be obtained. The distance between the centers of gravity of the open pores in the present disclosure is a linear distance connecting the centers of gravity of the open pores.

To measure the equivalent circle diameter of the open pores, a method called a particle analysis of the image analysis software is applied to the above measurement area as an object

As setting conditions for the distance between the center of gravity method and the particle analysis, for example, brightness is set to be dark, binarization method is set to be manual, a small figure removal area is set to be 1 µm², and a noise removal filter is set to be present, and then a threshold value should be set in such a way that a marker appearing on the screen matches the shape of the open pore. The threshold value is, for example, 155.

One of embodiments of a method for manufacturing the hermetic terminal of the present disclosure is described below.

A first tube body, a second tube body, and a ceramic substrate in which a conductive member is inserted into a through hole are prepared.

The ceramic substrate can be obtained by the following manufacturing method.

First, aluminum oxide powder, which is the main component, magnesium hydroxide, silicon oxide, calcium carbonate, and zirconium oxide powders, a dispersant to disperse the aluminum oxide powder as needed, and an organic binder are wet-mixed by a ball mill, a bead mill, or a vibration mill to obtain a slurry.

Here, the mean particle size (D₅₀) of the aluminum oxide powder is 3 um or less, preferably 1 um or less, and in a total of 100 mass% of the above-described powders, the content of the magnesium hydroxide powder is 0.87 mass% to 1.07 mass%, the content of the silicon oxide powder is 6.1 mass% to 7.5 mass%, the content of the calcium carbonate powder is 2.5 mass% to 3.1 mass%, and the content of the zirconium oxide is 1.0 mass% to 1.3 mass%.

The time for wet mixing is, for example, 40 to 50 hours. Examples of the organic binder include paraffin wax, wax emulsion (wax and emulsifier), PVA (polyvinyl alcohol), PEG (polyethylene glycol), and PEO (polyethylene oxide).

Next, the slurry obtained by the above-described method is spray-granulated to obtain granules, and then the granules are molded by a powder press molding method or a cold isostatic pressing method to obtain a molded body in a disk shape. Then, a ceramic substrate can be obtained by forming a through hole and step parts or a protrusion part by a cutting process, and sintering the molded body in which the through holes and the like are formed at a temperature of 1550°C or more and 1750°C or less.

To obtain a ceramic substrate provided with a plurality of open pores on the step surface where the metallized layer is included or on the tip end surface of the protrusion part, and where the value obtained by subtracting an average value of the equivalent circle diameters of the open pores from a distance between centers of gravity of the open pores is 20 um or more and 50 um or less, a molded body is manufactured by the cold isostatic pressing method with a molding pressure of 98 MPa or more and 147 MPa or less, and sintered at a temperature of 1580°C or more and 1750°C or less.

A coating layer composed of nickel, copper, or a copper-nickel alloy as a main component may be formed in advance on at least one of the connecting part of the conductive member with the ceramic substrate, the connecting part of the first tube body with the second tube body, the connecting part of the first tube body with the ceramic substrate, the connecting part of the second tube body with the first tube body, and the connecting part of the ceramic substrate with the first tube body by a plating method.

The above-described coating layer may be formed on the entire surface of each of the conductive member, the first tube body, and the second tube body.

If at least one of the end of the second tube body on the side of the first tube body and the end of the first tube body on the side of the second tube body includes a step surface, the above-described coating layer may be formed on the step surface.

In at least one of the connecting part of the ceramic substrate with the conductive member and the connecting part of the ceramic substrate with the first tube body the metallized layer may be formed in advance by a Mo-Mn method, and then a coating layer composed of nickel, copper or the copper-nickel alloy as a main component by the plating method.

The above-described coating layer may be formed on the entire outer peripheral surface of the ceramic substrate.

Then, by applying a brazing material including silver such as BAg-8, BAg-8A, BAg-8B as a main component to each of the opposing connecting parts and performing a heat treatment at an appropriate temperature, the connecting parts are connected, and the hermetic terminal of the present disclosure can be obtained.

Here, the appropriate temperature is the brazing temperature described in JIS Z 3281: 1998.

Further, to obtain a hermetic terminal provided with a flange, a first tube body, a ceramic substrate in which a conductive member is inserted into a through hole, and a second tube body to which a collar part is attached are prepared.

Then, after connecting each of the opposing connecting parts with the above-mentioned brazing material, the flange is attached to the outer peripheral side of the collar part, and the hermetic terminal of the present disclosure can be obtained by welding and fixing by the TIG (Tungsten Inert Gas) welding method.

The hermetic terminals of the present disclosure obtained by the above-mentioned manufacturing method have high embrittlement to hydrogen, and can therefore be used for a long period of time.

The present invention is not limited to the foregoing embodiment.

For example, in the above-described embodiment, an example that the second tube body 5 is connected to the flange 6 via the collar part 8 is shown, but the second tube body 5 may be directly connected to the flange 6. Further, in the above-described embodiment, an example that the collar part 8 has a U-shaped cross section is shown, but the collar part 8 may have another shape such as an L-shaped cross section or the like. If the collar part 8 has a U-shape, an L-shape, or the like, the bent part may be curved. Additionally, in the above-described embodiment, an example that the collar part 8 is connected to the second recessed part 6d of the flange 6 is shown, but the flange 6 may not include the second recessed part 6d, and the collar part 8 may be connected to the inner peripheral surface of the flange 6 or the main surface at the side of the second tube body 5.

### Description of the Reference Numeral

- 1: conductive member
- 2: through hole
- 3: ceramic substrate
- 3a: protrusion part
- 3b, 3c: main surface
- 4: first tube body
- 5: second tube body
- 6: flange
- 7: connecting layer
- 8: collar part
- 9: step part
- 10: metallized layer
- 20: hermetic terminal

## Claims

1. A hermetic terminal (20) comprising a plate-shaped ceramic substrate (3) provided with a through hole (2) for inserting a columnar conductive member (1) in a thickness direction, a first tube body (4) at surrounding the ceramic substrate, wherein the first tube body comprises a fernico-type alloy, an Fe-Ni alloy, an Fe-Ni-Cr-Ti-Al alloy, an Fe-Cr-Al alloy or an Fe-Co-Cr alloy, and **characterised by** further comprising a second tube body (5) coaxially connected with the first tube body, wherein the second tube body comprises an austenitic stainless steel with a nickel content of 10.4 mass% or more.

2. The hermetic terminal according to claim 1, wherein at least one of the end of the second tube body on the side of the first tube body and the end of the first tube body on the side of the second tube body has a step surface (4c, 5c).

3. The hermetic terminal according to claim 1 or 2, wherein the second tube body is provided with a coating layer (5d) composed of nickel, copper or a copper-nickel alloy as a main component at least on a connecting part with the first tube body.

4. The hermetic terminal according to any one of claims 1 to 3, wherein an inner peripheral surface of the first tube body is located outward rather than an outer peripheral surface of the second tube body.

5. The hermetic terminal according to any one of claims 1 to 4, further comprising a flange (6) connected to the outer peripheral surface of the second tube body and surrounding the second tube body.

6. The hermetic terminal according to claim 5, wherein the flange is provided with a second recessed part (6d) on the side of the second tube body, a collar part (8) having a U-shaped cross section along an axial direction of the second tube body is attached to the second recessed part, and the second tube body and the flange are connected to each other via the collar part, and wherein the flange is provided with a first recessed part (6c) at the side of the first tube body, and a connecting part between the ceramic substrate and the first tube body is located away from the second tube body than a bottom surface (6c1) of the first recessed part.

7. The hermetic terminal according to claim 6, wherein the collar part comprises an austenitic stainless steel with a nickel content of 10.4 mass% or more.

8. The hermetic terminal according to any one of claims 1 to 7, wherein a plurality of the conductive members are individually inserted into a plurality of the through holes, and the ceramic substrate is provided with step parts (9) recessed from at least one of the main surfaces around the through holes.

9. The hermetic terminal according to claim 8, wherein the ceramic substrate comprises the step parts recessed from both of the main surfaces around the through holes, one of the step parts is further provided with a metallized layer (10) on the step surface, and the step part on the side provided with the metallized layer is deeper than the step part on the side not provided with the metallized layer.

10. The hermetic terminal according to claim 9, wherein a depth of the step part (9a) on the side provided with the metallized layer is 45% or less of a thickness of the ceramic substrate.

11. The hermetic terminal according to any one of claims 1 to 7, wherein the plurality of conductive members are individually inserted into the plurality of through holes, and the ceramic substrate is provided with a protrusion part (3a) extending from at least one of the main surfaces around the through holes.

12. The hermetic terminal according to any one of claims 9 to 11, wherein the ceramic substrate is provided with a plurality of open pores on the step surface provided with the metallized layer or a tip end surface of the protrusion part, and a value obtained by subtracting an average value of equivalent circle diameters of the open pores from a distance between centers of gravity of the open pores is 20 um or more and 50 um or less.

## Patentansprüche

1. Hermetischer Anschluss (20), der aufweist: ein plattenförmiges Keramiksubstrat (3), das mit einem Durchgangsloch (2) zum Einsetzen eines säulenförmigen leitfähigen Elements (1) in einer Dickenrichtung bereitgestellt ist, einen ersten Rohrkörper (4), der das Keramiksubstrat umgibt, wobei der erste Rohrkörper eine Legierung des Fernico-Typs, eine Fe-Ni-Legierung, eine Fe-Ni-Cr-Ti-Al-Legierung, eine Fe-Cr-Al-Legierung oder eine Fe-Co-Cr-Legierung aufweist, und **dadurch gekennzeichnet, dass** er ferner einen zweiten Rohrkörper (5) aufweist, der koaxial mit dem ersten Rohrkörper verbunden ist, wobei der zweite Rohrkörper einen austenitischen rostfreien Stahl mit einem Nickelgehalt von 10,4 Massen-% oder mehr aufweist.

2. Hermetischer Anschluss gemäß Anspruch 1, wobei mindestens eines von dem Ende des zweiten Rohrkörpers auf der Seite des ersten Rohrkörpers und dem Ende des ersten Rohrkörpers auf der Seite des zweiten Rohrkörpers eine Stufenfläche (4c, 5c) aufweist.

3. Hermetischer Anschluss gemäß Anspruch 1 oder 2, wobei der zweite Rohrkörper zumindest an einem Verbindungsteil mit dem ersten Rohrkörper mit einer Überzugsschicht (5d) bereitgestellt ist, die aus Nickel, Kupfer oder einer Kupfer-Nickel-Legierung als Hauptkomponente zusammengesetzt ist.

4. Hermetischer Anschluss gemäß irgendeinem der Ansprüche 1 bis 3, wobei eine Innenumfangsfläche des ersten Rohrkörpers eher als eine Außenumfangsfläche des zweiten Rohrkörpers nach außen angeordnet ist.

5. Hermetischer Anschluss gemäß irgendeinem der Ansprüche 1 bis 4, ferner aufweisend einen Flansch (6), der mit der Außenumfangsfläche des zweiten Rohrkörpers verbunden ist und den zweiten Rohrkörper umgibt.

6. Hermetischer Anschluss gemäß Anspruch 5, wobei der Flansch mit einem zweiten Aussparungsteil (6d) auf der Seite des zweiten Rohrkörpers bereitgestellt ist, ein Kragenteil (8) mit einem U-förmigen Querschnitt entlang einer Axialrichtung des zweiten Rohrkörpers an dem zweiten Aussparungsteil angebracht ist und der zweite Rohrkörper und der Flansch über den Kragenteil miteinander verbunden sind, und wobei der Flansch mit einem ersten Aussparungsteil (6c) an der Seite des ersten Rohrkörpers bereitgestellt ist und ein Verbindungsteil zwischen dem Keramiksubstrat und dem ersten Rohrkörper von dem zweiten Rohrkörper weiter entfernt als eine Bodenfläche (6c1) des ersten Aussparungsteils angeordnet ist.

7. Hermetischer Anschluss gemäß Anspruch 6, wobei der Kragenteil einen austenitischen rostfreien Stahl mit einem Nickelgehalt von 10,4 Massenprozent oder mehr aufweist.

8. Hermetischer Anschluss gemäß irgendeinem der Ansprüche 1 bis 7, wobei eine Mehrzahl der leitfähigen Elemente einzeln in eine Mehrzahl der Durchgangslöcher eingesetzt ist und das Keramiksubstrat mit Stufenteilen (9) bereitgestellt ist, die von mindestens einer der Hauptflächen um die Durchgangslöcher herum ausgespart sind.

9. Hermetischer Anschluss gemäß Anspruch 8, wobei das Keramiksubstrat die Stufenteile aufweist, die von beiden der Hauptflächen um die Durchgangslöcher herum vertieft sind, wobei einer der Stufenteile ferner mit einer metallisierten Schicht (10) auf der Stufenfläche bereitgestellt ist und der Stufenteil auf der Seite, die mit der metallisierten Schicht bereitgestellt ist, tiefer als der Stufenteil auf der Seite ist, die nicht mit der metallisierten Schicht bereitgestellt ist.

10. Hermetischer Anschluss gemäß Anspruch 9, wobei eine Tiefe des Stufenteils (9a) auf der mit der metallisierten Schicht bereitgestellten Seite 45 % oder weniger einer Dicke des Keramiksubstrats beträgt.

11. Hermetischer Anschluss gemäß irgendeinem der Ansprüche 1 bis 7, wobei die Mehrzahl von leitfähigen Elementen einzeln in die Mehrzahl von Durchgangslöchern eingesetzt ist und das Keramiksubstrat mit einem Vorsprungsteil (3a) bereitgestellt ist, der sich von mindestens einer der Hauptflächen um die Durchgangslöcher herum erstreckt.

12. Hermetischer Anschluss gemäß irgendeinem der Ansprüche 9 bis 11, wobei das Keramiksubstrat mit einer Mehrzahl offener Poren auf der mit der metallisierten Schicht bereitgestellten Stufenfläche oder einer Spitzenendfläche des Vorsprungsteils bereitgestellt ist und ein Wert, der durch Subtrahieren eines Durchschnittswerts von äquivalenten Kreisdurchmessern der offenen Poren von einem Abstand zwischen Schwerpunkten der offenen Poren erhalten wird, 20 um oder mehr und 50 um oder weniger beträgt.

## Revendications

1. Borne hermétique (20) comprenant un substrat céramique (3) en forme de plaque pourvu d'un trou de passage (2) pour l'insertion d'un élément conducteur (1) en forme de colonne dans un sens d'épaisseur, un premier corps de tube (4) entourant le substrat céramique, le premier corps de tube comprenant un alliage de type fernico, un alliage Fe-Ni, un alliage Fe-Ni-Cr-Ti-Al, un alliage Fe-Cr-Al ou un alliage Fe-Co-Cr, et **caractérisée** en outre en comprenant un deuxième corps de tube (5) connecté coaxialement au premier corps de tube, le deuxième corps de tube comprenant un acier inoxydable austénitique avec une teneur en nickel de 10,4 % en masse ou plus.

2. Borne hermétique selon la revendication 1, dans laquelle au moins l'une parmi l'extrémité du deuxième corps de tube sur le côté du premier corps de tube et l'extrémité du premier corps de tube sur le côté du deuxième corps de tube a une surface en gradin (4c, 5c).

3. Borne hermétique selon la revendication 1 ou 2, dans laquelle le deuxième corps de tube est pourvu d'une couche de revêtement (5d) composée de nickel, de cuivre ou d'un alliage cuivre-nickel comme composant principal au moins sur une partie de connexion avec le premier corps de tube.

4. Borne hermétique selon l'une quelconque des revendications 1 à 3, dans laquelle une surface périphérique intérieure du premier corps de tube est située vers l'extérieur plutôt qu'une surface périphérique extérieure du deuxième corps de tube.

5. Borne hermétique selon l'une quelconque des revendications 1 à 4, comprenant en outre une bride (6) reliée à la surface périphérique extérieure du deuxième corps de tube et entourant le deuxième corps de tube.

6. Borne hermétique selon la revendication 5, dans laquelle la bride est pourvue d'une deuxième partie en retrait (6d) sur le côté du deuxième corps de tube, une partie de col (8) ayant une section transversale en forme de U le long d'une direction axiale du deuxième corps de tube est fixée à la deuxième partie en retrait, et le deuxième corps de tube et la bride sont connectés l'un à l'autre par l'intermédiaire de la partie de col, et dans laquelle la bride est pourvue d'une première partie en retrait (6c) sur le côté du premier corps de tube, et une partie de connexion entre le substrat céramique et le premier corps de tube est située plus loin du deuxième corps de tube qu'une surface inférieure (6c1) de la première partie en retrait.

7. Borne hermétique selon la revendication 6, dans laquelle la partie de col comprend un acier inoxydable austénitique avec une teneur en nickel de 10,4 % en masse ou plus.

8. Borne hermétique selon l'une quelconque des revendications 1 à 7, dans laquelle une pluralité des éléments conducteurs sont insérés individuellement dans une pluralité des trous de passage, et le substrat céramique est pourvu de parties en gradin (9) en retrait d'au moins une des surfaces principales autour des trous de passage.

9. Borne hermétique selon la revendication 8, dans laquelle le substrat céramique comprend les parties en gradin en retrait des deux surfaces principales autour des trous de passage, l'une des parties en gradin est en outre pourvue d'une couche métallisée (10) sur la surface en gradin, et la partie en gradin sur le côté pourvu de la couche métallisée est plus profonde que la partie en gradin sur le côté qui n'est pas pourvu de la couche métallisée.

10. Borne hermétique selon la revendication 9, dans laquelle une profondeur de la partie en gradin (9a) sur le côté pourvu de la couche métallisée est 45% ou moins d'une épaisseur du substrat céramique.

11. Borne hermétique selon l'une quelconque des revendications 1 à 7, dans laquelle la pluralité d'éléments conducteurs sont insérés individuellement dans la pluralité de trous de passage, et le substrat céramique est pourvu d'une partie saillante (3a) s'étendant à partir d'au moins l'une des surfaces principales autour des trous de passage.

12. Borne hermétique selon l'une quelconque des revendications 9 à 11, dans laquelle le substrat céramique est pourvu d'une pluralité de pores ouverts sur la surface en gradin pourvue de la couche métallisée ou une surface d'extrémité de pointe de la partie saillante, et une valeur obtenue en soustrayant une valeur moyenne de diamètres de cercle équivalents des pores ouverts d'une distance entre des centres de gravité des pores ouverts est de 20 um ou plus et de 50 um ou moins.
